

# UNITED STATES PATENT OFFICE.

ELIEL L. SHARPNECK, OF BAKERSFIELD, CALIFORNIA, ASSIGNOR TO ROMANITE COMPANY OF AMERICA, OF BOSTON, MASSACHUSETTS, A TRUST OF MASSACHUSETTS.

## PLASTIC COMPOSITION.

1,315,342.

Specification of Letters Patent.

Patented Sept. 9, 1919.

No Drawing.

Application filed December 27, 1917. Serial No. 209,106.

*To all whom it may concern:*

Be it known that I, ELIEL L. SHARPNECK, a citizen of the United States of America, and a resident of Bakersfield, in the county 5 of Kern and State of California, have invented a new and useful Plastic Composition, of which the following is a specification.

The object of this invention is to provide 10 an improved composition that can be used for paving roadways, streets, and sidewalks; for reservoir-linings, and for any purpose where the material used must resist the effect of great wear, as well as that of heat, 15 cold and moisture.

The composition comprises a finely di- 20 vided filler composed of any soil, sand, earthy matter, or mixture thereof, a mineral asphaltic binder, sulfate of aluminum, also powdered limestone, for instance in the form 25 of dolomite or marble dust.

The filler which forms approximately 30% to 85% of the whole amount, is screened so that it is a uniformly fine mass. This 25 is heated and thoroughly dried to remove all moisture before being mixed. In mixing, the filler is heated to about 300° F., and to this is added from 7% to 15% mineral asphalt binder, also heated to the same de- 30 gree, the amount used depending on what amount the filler will absorb. Approximately 2% of sulfate of aluminum is added while heating. About 6% of powdered limestone, as for instance, dolomite or 35 marble dust, may be also added while heat- ing. If it was simply a question of making the composition hard, it would be only nec- essary to add sulfur to the composition, but sulfur also makes it brittle, as well as hard,

40 and I find that sulfate of copper, while it tempers or hardens the asphaltum, leaves it in a more or less brittle condition. The sulfate of aluminum, however, hardens the asphaltum, and also renders it very tough 45 and not brittle, so that the composition when acted upon by the sulfate of aluminum has a toughness like rubber which is of greater importance and value in paving roads and streets as it prevents the cracking of the

50 surface which is bound to occur if the composition is brittle. I prefer to use the lime- stone in the form of marble dust, inasmuch as this marble dust when incorporated in the composition makes the composition more 55 dense and more impervious to moisture and

also acts to harden the mass to a certain ex- tent. The asphaltum used is of 50 to 60 penetration.

The composition is particularly designed 60 for use for paving purposes and when the composition is thoroughly mixed, it may be molded to form blocks, or it may be spread in a uniform layer over the roadway and then rolled with a relatively light roller. After this, a relatively heavier roller is used 65 and the rolling continued until no further compression is shown under the roller. It is to be understood that in laying pav- 70 ements, a foundation course of about 3" thick and a wearing surface of about 2" in thickness are used, the wearing surface or layer being laid upon the foundation course after the latter has been rolled. The wearing layer is spread over the founda- 75 tion layer or course at about 300° F. and when rolled the two courses or layers will 80 fuse together in one inseparable unit from curb to curb. The use of aluminum sulfate hardens, toughens and strengthens the asphalt and the entire paving mixture, so 85 that it is rendered strong and absolutely immune to heat, cold and moisture, and pre- 90 vents it from cracking or getting soft. Marble dust, limestone, or dolomite can be used as desired, as dolomite is a variety of magnesian limestone. This crushed lime- 95 containing rock assists in making the mass more dense by its chemical action when combined with asphalt and sulfate of aluminum. Of course, when I refer to sulfate of alu- 100 minum, I include such an ingredient as alum, as the latter is a double sulfate of aluminum with certain other elements.

I am aware that it has been heretofore proposed to use sulfate of copper in combi- 105 nation with an earthy filler and asphaltum. The action of the copper salt is to harden the asphaltum. There is an oxidizing effect, due to the withdrawal of hydrogen from the hydrocarbon colloids and dispersoids, 110 which make up the body and give character to all asphalts. Copper sulfate crystallizes with four molecules of water and when the salt is introduced into a hot asphalt batch at approximately 300° to 400° F., the water of crystallization is at once liberated, the water producing a foamy condition of the asphalt, which is advantageous and takes part in the hardening reactions immediately occur- 115 ring. I have found by actual tests, however,

that a much better effect is secured by using crude aluminum sulfate, which hardens the asphalt to a hardness more than twice that produced by copper sulfate. Whereas copper sulfate contains four molecules of water of crystallization, aluminum sulfate contains eighteen molecules, so that on heating this compound, the aluminum sulfate melts in its own water of crystallization, which is not the case with copper sulfate. Thus, an even distribution of the aluminum sulfate is secured throughout the asphaltic mixture immediately upon the addition of the aluminum sulfate. Weight for weight, the aluminum sulfate will produce twice as much result as copper sulfate and at a much lower cost.

Having thus described my invention, what I claim as new therein and desire to secure 20 by Letters Patent is:—

1. A plastic composition comprising a relatively large proportion of a finely divided, earthy filler, mineral asphalt, and sulfate of aluminum intimately combined therewith.

2. A plastic composition comprising a relatively large proportion of a finely divided, earthy filler, mineral asphaltum, sulfate of aluminum intimately combined

therewith while in a highly heated condition, and finely crushed limestone.

3. A plastic composition comprising 80 to 85% of a finely divided, earthy filler, mineral asphaltum, and sulfate of aluminum.

4. A plastic composition comprising 80 to 85% of a finely divided, earthy filler, mineral asphalt, sulfate of aluminum, and finely crushed limestone.

5. A plastic composition comprising 80 to 85% of finely divided filler, 12 to 7% of mineral asphalt, about 2% of sulfate of aluminum, and about 6% of finely crushed limestone.

6. A method of forming a plastic composition consisting in heating a finely divided filler to a temperature of approximately 300° F., adding thereto a mineral asphaltic binder heated to the same degree, and sulfate of aluminum and stirring the mass while heated until agitation ceases.

In witness whereof, I have hereunto signed my name in the presence of two subscribing witnesses.

ELIEL L. SHARPNECK. [L. S.]

Witnesses:

IRMA V. MYER,

Mrs. E. L. SHARPNECK.